

## UNITED STATES PATENT OFFICE

2,064,301

METHOD OF PRODUCING A BRONZE FINISH  
ON COPPER AND COPPER ALLOYS

John R. Freeman, Jr., Cheshire, and Rollo L. Hungerford, Waterbury, Conn., assignors to The American Brass Company, Waterbury, Conn., a corporation of Connecticut

No Drawing. Application November 10, 1934,  
Serial No. 752,476

4 Claims. (Cl. 148—6)

This invention relates to copper and copper alloys, and has for an object to provide an improved method of producing a bronze finish on copper or copper alloys so as to give articles made of such materials a weathered bronze appearance in a short time.

We are aware of the patent to Laist et al No. 1,428,170 granted September 5, 1922 in which is disclosed a process for coloring metallic copper to secure a colored surface of various shades of green and blue, by immersing the copper article in a solution of copper nitrate and copper chloride, and then washing and treating with various solutions to make the colored coating more adherent and less soluble.

In our process, however, we do not wish a colored coating, but secure a rich weathered bronze surface appearance which is very attractive.

20 In carrying out our method the articles of copper or copper alloy are cleaned free from scale, grease, dirt, or any similar surface imperfection. We then immerse the article in a hot concentrated solution of copper nitrate, 25 or otherwise subject it to the action of such solution, for such a period of time as experience has shown to be desirable. This is ordinarily from about five minutes to a half hour, depending on the temperature of the solution and the 30 alloy used, ordinarily about 15 minutes with a solution temperature of 80° to 90° C. has proven very satisfactory. The specimen is now washed in hot water, preferably at a temperature of about 80° to 100° C., and the specimen is then 35 dried. The specimen now has upon its surface a roughly adhering green salt consisting of basic copper nitrate under which is a hard adherent surface film of a mixture of cuprous and cupric oxides which has a desirable weathered 40 bronze appearance.

We have found that this green loosely adhering layer of basic salt can be readily removed by a buffing operation which also gives to the underlying surface film of cupric and cuprous 45 oxides a fine bronze sheen. The buffing operation is preferably performed with a soft cloth buffing wheel.

This process produces a very beautiful weathered bronze appearance on copper and copper alloys, and has been found to give a particularly desirable appearance on such copper alloys as the silicon bronzes of the so-called "Everdur"

type, such for example as those containing from about .1 to 10% silicon and up to 4 or 5% manganese, and similar alloys. It is, however, not confined to such alloys, but is adapted for treating copper and copper alloys in general. 5

Having thus set forth the nature of our invention, what we claim is:

1. A method of producing a weathered bronze coating or finish on articles of copper and copper alloys which comprises immersing the article in a hot concentrated solution of predominantly copper nitrate to form on the metal a surface film of copper oxide under copper salts, washing in hot water to loosen the copper salts, drying, and then buffing the surface in such 15 manner as to remove the salts and impart to the oxide film a weathered bronze appearance.

2. A method of producing a weathered bronze coating or finish on articles of copper and copper alloys comprising subjecting the article to 20 the action of a hot concentrated solution of predominantly copper nitrate to form a surface film of copper oxide and adhering copper salts, washing the article in hot water to loosen the copper salts and then drying, and then buffing 25 the surface in such manner as to remove the salts and impart a bronze finish to the copper oxides.

3. In a method of producing a weathered bronze coating or finish on articles of copper 30 and copper alloys, the steps which consist in subjecting the article to the action of a hot concentrated solution predominantly of copper nitrate to produce thereon a coating of a green salt overlying a surface film of copper oxides, 35 washing in hot water to loosen the green salt and drying, and then buffing the surface in such manner as to remove the colored salts and impart a bronze finish to the oxides.

4. A method of producing a weathered bronze 40 coating or finish on articles of copper and copper alloys comprising cleaning the article and subjecting it to a hot concentrated solution of predominately copper nitrate for a sufficient time to produce on its surface a roughly adhering salt of basic copper nitrate over a surface film of copper oxides, then washing the article in hot water to loosen the salt and drying, and 45 buffing the surface to remove the salt and impart a bronze finish to the oxide film. 50

JOHN R. FREEMAN, JR.  
ROLLO L. HUNGERFORD.